

## UNITED STATES PATENT OFFICE

2,450,224

METHOD OF PREPARATION OF BARIUM  
SOAP GREASES

Eric A. Bergmann, Fishkill, N. Y.; Harry V. Ashburn, Waynesburg, Pa.; and George W. Eckert, Glenham, N. Y., assignors to The Texas Company, New York, N. Y., a corporation of Delaware

No Drawing. Application December 6, 1946,  
Serial No. 714,640

7 Claims. (Cl. 252-39)

1

This invention relates to improvements in the manufacture and production of lubricating grease compositions and particularly to improvements in the manufacture of stable barium soap greases.

Although barium soap greases have been recognized as a desirable adjunct to the more conventional line of lubricating greases by virtue of their inherent properties of water resistance and comparatively high dropping points, their general application has been retarded because of the alleged limitations in composition and attendant difficulties in manufacture. Prior investigators have concluded that the desirable characteristics of barium soap greases are attained by the basic and/or complex barium soap greases which can only be prepared by a complicated method of manufacture involving intricate compounding procedures and special cooling and milling operations. It has been the experience of the prior art that the preparation of the normal barium soap greases was even more difficult and required water for stabilization, which substantially nullified any improvement over the conventional calcium soap greases.

It has now been found possible to prepare barium soap greases by a simple and economical method which avoids the use of complicated manufacturing techniques and can easily be carried out in conventional steam-heated equipment. Although this discovery may be generally applied to all barium soap greases, including the mixed-base greases in which barium is one of the metal components, it is particularly applicable to the normal barium soap greases and affords a method of preparing a stable, normal barium soap grease without the aid of water or other added stabilizers.

This improved method of preparing barium soap greases is dependent upon two important features of the invention, namely, the presence of a naphthenic oil during the saponification of the fatty acid material and the stirring down of the dehydrated grease base while cooling to a temperature below the critical transition temperature of the grease base.

Since there is no clear line of demarcation between naphthenic and paraffinic oils and the naphthenicity or paraffinicity of an oil is a matter of degree, reference will be made to the viscosity gravity constant (VGC) of the oil. The VGC is an arbitrary constant calculated from the Saybolt Universal viscosity and the specific gravity of an oil, the value of which increases with naphthenicity and decreases with paraffinicity (Hill & Coats, Ind. & Eng. Chem., vol. 20, 1928, pp.

2

641-4). Relating the VGC to the process of the invention it was found that the saponification should be conducted in the presence of a naphthenic oil possessing a VGC of at least 0.870.

It was also found that upon cooling the barium soap base following dehydration the structure of the base undergoes a complete phase change. This transition of structure is manifested in the appearance of the grease base which changes from a homogeneous gel-like structure to an inhomogeneous dry crumbly mass. The particular temperature range over which this transition occurs is dependent upon and varies with the acid component of the barium soap and will be referred to in the following description and the claims as the critical transition temperature of the grease base. At this critical transition temperature the grease base loses its grease structure and if worked up in the conventional manner, would result in an inhomogeneous product that cannot be brought together even after extensive milling. This may be avoided, however, by maintaining the concentration of the barium soap in the grease base at least greater than approximately 40% and continuously stirring the dehydrated base while cooling through the critical transition temperature range until the grease base reverts back to a homogeneous taffy structure.

According to the process of the invention barium soap greases may be prepared by saponifying a soap-forming fatty acid with barium hydroxide or hydrate in the presence of a naphthenic mineral oil possessing a viscosity gravity constant (VGC) of at least 0.870 to effect solvation of the resulting barium soap. The saponification product is then dehydrated at a temperature not in excess of the melting point of the soap base and preferably at temperatures of approximately 300 to 320° F. After dehydration is substantially complete the product is cooled with continuous stirring without the addition of substantial amounts of lubricating oil. The stirring down of the dehydrated soap base is continued until a complete phase change in the soap base structure has been obtained. This phase change or transition of the soap structure is usually completed at around 200° F. It is particularly desirable to maintain the soap concentration at least greater than approximately 40% and preferably around 50% during the stirring down and cooling operation.

The appearance of the grease base structure will vary somewhat with the type of fatty acid used for saponification. When using the con-

ventional saturated fatty acids as the acid component of the soap base a tough rubbery gel is obtained on dehydration which then changes on stirring and cooling to a dry crumbly mass and finally comes around to a tough sticky mass. It is requisite that this complete transition of structure be completed before any substantial addition of lubricating oil since oil addition at any point prior to the complete transition results in an inhomogeneous grease containing hard soap lumps which cannot be brought together. After the completion of the phase change of the grease structure, the mineral lubricating oil may be incorporated until the desired consistency is reached and the final grease composition drawn from the kettle.

Throughout the preparation of the grease composition it is desirable to maintain continuous stirring. During the cooling stage, when the concentration of the soap is approximately 50% or greater considerable load is applied to the stirring mechanism and if the stirring mechanism becomes overloaded it may be desirable to incorporate small amounts of the mineral lubricating oil to reduce the load on the stirring mechanism. The addition of the mineral oil at this stage should be controlled so that the concentration of the soap is not reduced to substantially below 40%.

Although any conventional fatty acid material may be used as the acid component of the barium soap, the best yields and quality of grease are obtained by charging fatty acids or mixtures thereof and particularly fatty acids containing at least 16 carbon atoms or predominating amounts of fatty acids of at least 16 carbon atoms. Glycerides such as are contained in the natural fats may be used provided the free glycerin formed on saponification is substantially removed by steam distillation or by prolonged heating in the dehydration stage. Examples of the fatty acids found suitable for the preparation of the barium greases include such acids as stearic, palmitic, behenic, oleic, hydroxy stearic, etc.

As has been previously mentioned, a naphthenic mineral oil possessing a VGC of at least 0.870 is required to effect solvation of the barium soap formed in the saponification stage of the process. This naphthenic mineral oil may be either a distillate or residual lubricating oil of the desired viscosity or may consist of a blend of lubricating oils in which the VGC of the final blend is at least 0.870. The amount of the naphthenic mineral oil charged in the saponification stage is not critical to the invention but for ease of manufacture it is preferable to employ approximately an equal weight of mineral oil based upon the weight of the fatty acids charged. After the saponification further processing and finishing of the grease base may be conducted with any of the conventional lubricating oils, irrespective of the naphthenicity or paraffinicity of the oil.

Contrary to the experiences of the prior art the process of the invention permits the preparation of stable barium soap greases and particularly normal barium soap greases without limitations in composition requiring the addition of water or the presence of free fatty acid to effect stability. According to the present process barium soap greases can be prepared neutral or containing free acid or free alkali, as desired, without producing any adverse effect on the stability of the product.

The following example is presented as an il-

lustration of the method of preparing a normal barium soap grease in accordance with the process of the invention.

*Example*

5 310 grams of 90% stearic acid and 372 grams of a naphthenic Pale Oil possessing a S. U. V. at 100° F. of 312 and a VGC of 0.884 were charged to a grease kettle. The stearic acid was melted at 210° F., at which temperature 563 grams of a hot aqueous solution of barium hydroxide (17.6% Ba(OH)<sub>2</sub>) were added followed by 50 ml. of water. This mixture was stirred at 210° F. for one-half hour after all the water had evaporated. The temperature was then raised to 310° F. in 25 minutes and held at this temperature for 15 minutes, at which point the grease base was a stiff, taffy-like mass and rather rubbery. The heat was then removed and the mass stirred with natural cooling, the temperature reaching 200° F. in approximately 1 hour and 50 minutes. During the cooling period the appearance of the grease base changed from a stringy, taffy-like mass to a dry and flaky mass at about 240° F. 20 Further cooling and stirring resulted in a stiff, grainy dough at about 230° F., which became a smooth, pasty mass entirely devoid of lumps, as the temperature decreased. The grease base was maintained at 200° F. for about 15 minutes, 25 after which 1928 grams of Pale Oil was gradually incorporated with continuous stirring. After the oil addition was complete the grease composition was stirred an additional 15 minutes and the transparent reddish grease withdrawn from the kettle. The tests on the final grease composition were as follows:

|                                                              |      |
|--------------------------------------------------------------|------|
| Barium soap, percent (calculated)                            | 14.0 |
| Free alkali (as Ba(OH) <sub>2</sub> ), per cent <sup>1</sup> | 0.08 |
| Free fatty acid (as oleic), per cent <sup>1</sup>            | 0.10 |
| 40 Dropping point, °F (ASTM)                                 | 293  |
| Penetration, 77 °F. (ASTM):                                  |      |
| Unworked                                                     | 207  |
| Worked                                                       | 277  |

45 <sup>1</sup> "The Institute Spokesman," National Lubricating Grease Institute, January, 1944. "Test Methods for Determining Free Acid and Free Alkali in Greases."

Obviously many modifications and variations of the invention, as hereinbefore set forth, may be made without departing from the spirit and scope thereof and, therefore, only such limitations should be imposed as are indicated in the appended claims.

We claim:

55 1. A method of preparing a normal barium soap grease composition which comprises saponifying a soap-forming fatty acid with not more than the stoichiometric equivalent of barium hydrate in the presence of a mineral oil possessing a VGC of at least 0.870 to produce a saponification product of normal barium soap, dehydrating the saponification product at temperatures not in excess of the melting point of the soap base, cooling the dehydrated product with continuous stirring to a temperature below the critical transition temperature of the grease base without reducing the concentration of the soap component to substantially below 40%, thereafter adding mineral lubricating oil to obtain the desired consistency and drawing the resulting grease composition.

60 2. A method of preparing a normal barium soap grease composition which comprises saponifying a fatty acid containing at least 16 carbon atoms with substantially the stoichiometric

quantity of barium hydrate in the presence of a mineral oil possessing a VGC of at least 0.870 to produce a saponification product of normal barium soap, dehydrating the saponification product at temperatures not in excess of the melting point of the soap base, cooling the dehydrated product with continuous stirring to a temperature of approximately 200° F. without reducing the concentration of the soap component to substantially below 40%, thereafter adding mineral lubricating oil to obtain the desired consistency and drawing the resulting grease composition.

3. A method of preparing a normal barium soap grease composition which comprises saponifying a fatty acid containing at least 16 carbon atoms with barium hydrate, in stoichiometric quantities required for the preparation of a normal barium soap, in the presence of a mineral oil possessing a VGC of at least 0.870, dehydrating the saponification product at temperatures not in excess of the melting point of the soap base, cooling the dehydrated product with continuous stirring to a temperature below the critical transition temperature of the normal soap base without reducing the concentration of the normal soap component to substantially less than 40%, thereafter adding mineral lubricating oil to obtain the desired consistency and drawing the finished grease composition.

4. A method of preparing a normal barium soap grease composition which comprises saponifying a fatty acid containing at least 16 carbon atoms with substantially the stoichiometric quantity of barium hydrate in the presence of sufficient mineral lubricating oil possessing a VGC of at least 0.870 to effect solvation of the resulting normal barium soap, dehydrating the saponification product at temperatures of approximately 300-320° F., cooling the dehydrated product with continuous stirring to a temperature of approximately 200° F. without reducing the concentration of the soap component to substantially below 40%, thereafter adding mineral lubricating oil to obtain the desired consistency and drawing the resulting grease composition.

5. A method of preparing a normal barium soap grease composition which comprises saponifying a fatty acid containing at least 16 carbon atoms with not more than the stoichiometric equivalent of barium hydrate in the presence of approximately equal weights, based upon the weight of fatty acid, of a mineral oil possessing a VGC of at least 0.870 to produce an oil solution of normal barium soap dehydrating the saponification product at temperatures not in excess of the melting point of the soap base, cooling the dehydrated product with continuous

stirring to a temperature of approximately 200° F. without reducing the concentration of the soap component to substantially below 40%, thereafter adding mineral lubricating oil to obtain the desired consistency and drawing the resulting grease composition.

6. A method of preparing a normal barium stearate grease composition which comprises saponifying stearic acid with not more than the stoichiometric equivalent of barium hydrate in the presence of a mineral oil possessing a VGC of at least 0.870 to produce normal barium stearate, dehydrating the saponification product at temperatures not in excess of the melting point of the soap base, cooling the dehydrated product with continuous stirring to a temperature of approximately 200° F. without reducing the concentration of the barium stearate to substantially below 40%, adding mineral lubricating oil to obtain the desired consistency and drawing the resulting grease composition.

7. A method of preparing a normal barium stearate grease composition which comprises saponifying stearic acid with substantially the stoichiometric quantity of barium hydrate in the presence of about an equal quantity based on the stearic acid of a mineral lubricating oil possessing a VGC of at least 0.870 to produce an oil solution of normal barium stearate, dehydrating the saponification product at temperatures above 300° F. but not in excess of the melting point of the soap base, cooling the dehydrated product with continuous stirring to a temperature of approximately 200° F. without reducing the concentration of the barium stearate to substantially below 50%, thereafter adding mineral lubricating oil to obtain the desired consistency and drawing the resulting grease composition.

ERIC A. BERGMANN.  
HARRY V. ASHBURN.  
GEORGE W. ECKERT.

#### REFERENCES CITED

The following references are of record in the file of this patent:

#### UNITED STATES PATENTS

| Number    | Name                  | Date          |
|-----------|-----------------------|---------------|
| 2,033,148 | Ott, et al. -----     | Mar. 10, 1936 |
| 2,070,781 | Brunstrum, et al. --- | Feb. 16, 1937 |
| 2,154,383 | Ott, et al. -----     | Apr. 11, 1939 |
| 2,417,433 | McLennan -----        | Mar. 18, 1947 |

#### OTHER REFERENCES

55 McLennan, Methods of Compounding Barium Greases, Their Properties, Uses and Future—Article in National Petroleum News, April 5, 1944, pages R 234, R 236, R 238, and R 239.